

## UNITED STATES PATENT OFFICE

2,197,834

## MINERAL OIL COMPOSITION

Orland M. Reiff, Woodbury, John J. Giannmaria, Riverside, and Horace E. Redman, Woodbury, N. J., assignors to Socony-Vacuum Oil Company, Incorporated, New York, N. Y., a corporation of New York

No Drawing. Application May 26, 1938,  
Serial No. 210,160

28 Claims. (Cl. 87—9)

This invention has to do in a general way with mineral oil compositions and is more particularly related to compositions comprised of mineral oil and a minor proportion of an added ingredient which will improve the oil in one or more important respects.

It is well known to those familiar with the art that mineral oil fractions refined for their various uses are in and of themselves usually deficient in one or more respects, so that their practical utility is limited even in the particular field for which they have been refined. For example, mineral oil fractions refined for use as lubricants have a tendency to oxidize under conditions of use with the formation of sludge or acidic oxidation products; also the lighter fractions such as gasoline and kerosene tend to oxidize with the formation of color bodies, gum, etc. In order to prevent the formation of these products and thereby extend the useful life of the oil fraction, it is common practice to blend with such oil fractions an additive ingredient which will have the effect of inhibiting oxidation, such ingredients being generally known to the trade as oxidation inhibitors or sludge inhibitors, gum inhibitors, etc.

It is also the practice to add other ingredients to mineral oil fractions for the purpose of improving "oiliness" characteristics and the wear-reducing action of such mineral oils when they are used as lubricants, particularly when the oils are used for the purpose of lubricating metal surfaces which are engaged under extremely high pressures and at high rubbing speeds.

Other ingredients have been developed for the purpose of depressing the pour point of mineral oil fractions which have been refined for use as lubricants, such refinement leaving a certain amount of wax in the oil, which, without the added ingredient, would tend to crystallize at temperatures which render the oil impracticable for use under low temperature conditions. Additive agents have also been developed for improving the viscosity index of lubricating oil fractions. In the case of internal combustion engines, particularly those operating with high cylinder pressures, there is a decided tendency for the ordinary lubricating oil fractions to form, under such conditions of use, carbonaceous deposits which cause the piston rings to become stuck in their slots and which fill the slots in the oil ring or rings,

thus materially reducing the efficiency of the engine. Ingredients have therefore been developed which, when added to the oil, will reduce the natural tendency of the oil to form deposits which interfere with the function of the piston rings.

Aside from the corrosive action which attends the formation of acidic products of oxidation in mineral oil fractions of the lubricant range, it has been discovered that certain types of recently developed hard metal alloy bearing metals, such as cadmium-silver alloy bearings, are attacked by ingredients in certain types of oils, particularly oils of high viscosity index obtained by various methods of solvent refining. This corrosive action on alloys of the above type has led to the development of corrosion inhibitors which may be used in solvent-refined oils to protect such bearing metals against this corrosive action.

In the lighter mineral oil fractions, such as those used for fuel purposes, particularly in internal combustion engines, it has been found that the combustion characteristics of the fuel may be controlled and improved by adding minor proportions of various improving agents thereto.

The various ingredients which have been developed for use in mineral oil fractions to improve such fractions in the various respects enumerated above are largely specific to their particular applications, and it has therefore been the practice to add a separate ingredient for each of the improvements which is to be effected.

It is a primary object of the present invention to provide a mineral oil composition which has been improved in one or more of the various properties enumerated above by the incorporation therein of a small quantity of a multifunctional compound selected from that group or class of metal-organic compounds which may be designated as the oil-soluble or oil-miscible metal salts of alkyl-substituted hydroxyaromatic carboxylic acids in which both the hydroxyl and the carboxyl hydrogens are substituted with metal. We have discovered that metal oxyaromatic-metal carboxylate salts of the general class above referred to may be added in small quantities to mineral oil fractions to form mineral oil compositions or blends superior to the unblended fractions in one or more important respects, and the present invention, therefore, is broadly directed to

a mineral oil composition containing a compound falling into the general class referred to.

The oil-improving agents contemplated by this invention are all characterized by the presence of an aromatic nucleus in which at least one nuclear hydrogen has been substituted with a metal-oxy group and another nuclear hydrogen is substituted with a carboxyl group in which the carboxyl hydrogen has been replaced with its equivalent weight of metal. This characterizing group may be represented by the formula:



in which  $T'$  represents an aromatic nucleus;  $(OM)$  represents at least one hydroxyl group the hydrogen of which is replaced by its equivalent weight of metal  $M$ ; and  $COOM'$  represents at least one carboxyl group in which the hydrogen is replaced with its equivalent weight of a metal,  $M'$ , which may be the same as, or different from, the metal  $M$ . Both the  $(OM)$  group and the  $(COOM')$  group are attached to the nucleus  $T'$ .

The metal salts of hydroxyaromatic carboxylic acids of the type corresponding to the group represented by the above formula which are otherwise unsubstituted are not miscible with mineral oil, and it is therefore important that the improving agents containing the above characterizing group have additional nuclear hydrogen replaced with substituents of a solubilizing nature. In other words, it is important that the aryl nucleus carry a substituent or substituents which will render the composition as a whole miscible with mineral oil fractions. By the terms "oil-miscible" or "oil-soluble" as they are used herein we have reference to that property of remaining uniformly dispersed in the mineral oil fraction either as a true solution or as a colloidal suspension during normal conditions of handling and use.

The improving agents contemplated by this invention are characterized by the presence of alkyl substituents in the aryl nucleus, and the improving agents preferred for use in viscous mineral oils are further characterized by the presence of alkyl or aliphatic substituents in the aryl nucleus which will give other properties to the composition as a whole in addition to oil-miscibility. We have found, for example, that where the aryl nucleus is substituted with one or more aliphatic groups corresponding to certain aliphatic hydrocarbon compounds of relatively high molecular weight (herein referred to as heavy alkyl groups), a compound or composition can be obtained which will effect marked improvement in the viscosity index and the pour point as well as other important properties of viscous mineral oils.

As a general proposition, therefore, it may be said that the improving agents contemplated by this invention are metal salts of hydroxyaromatic carboxylic acid having the characterizing group  $T'(OM)(COOM')$  described above, in which additional nuclear hydrogen is replaced with an oil-solubilizing substituent such as a predominantly aliphatic material, such substituent comprising a sufficient proportion of the composition as a whole to render the same miscible with mineral oil fractions under normal conditions of handling and use. As a further generalization it may be said that at least one point on the aromatic nucleus  $T'$ , and preferably two or more points on such nucleus, are substituted with aliphatic hydrocarbon radicals or groups, such aliphatic rad-

icals or groups preferably being high molecular weight derivatives or heavy alkyl groups.

The simplest type of compound satisfying the above requisites may be represented by the formula:



in which  $R$  represents at least one aliphatic hydrocarbon radical or group, such group or groups preferably corresponding to relatively high molecular weight aliphatic hydrocarbons and being attached to a mono or poly cyclic aromatic nucleus  $T$  and in which  $(OM)$  and  $(COOM')$  are as indicated above.

In addition to the aliphatic or alkyl substituent  $R$ , the compounds or compositions contemplated herein as mineral oil improving agents may have additional nuclear hydrogen replaced with other substituents which may or may not have a solubilizing effect upon the composition as a whole. Such a compound in its simplest form may be represented by the formula:



in which  $R$ ,  $T$ ,  $(OM)$ , and  $(COOM')$  have the same significance indicated above and in which  $Y$  represents residual hydrogen which may be replaced by a radical from the group consisting of: chlorine, alkoxy, aroxy, aralkyl, alkaryl, aryl, nitro, and amino radicals or groups. Compounds of the above general formula-type having mono, di, and tri cyclic nuclei are illustrated by the following specific formulae:



in which at least one  $R'$  represents an aliphatic radical or group, preferably a heavy alkyl group, and in which the remaining  $R'$ 's represent residual hydrogen which may be replaced with hydroxy, chlorine, alkoxy, aroxy, aralkyl, alkaryl, aryl, nitro and amino radicals or groups.

In the foregoing examples it will be observed that the aliphatic or alkyl substituent is a monovalent aliphatic hydrocarbon group, but, as will appear from the hereinafter described synthesis of our oil-improving agent, part or all of the aliphatic hydrocarbon material may be comprised of polyvalent aliphatic hydrocarbon radicals or groups in which the several valences are attached to separate aromatic nuclear groups. Compounds of this type are included under the following general formula representation:



in which  $T$ ,  $(OM)$ , and  $(COOM')$  have the same significance indicated above;  $R^v$  represents at least one aliphatic or alkyl radical or group, such alkyl group or groups being attached by one valence only to at least one aromatic nucleus  $T$ ,  $v$  representing the valence of the aliphatic radical  $R^v$ , which may be one to four;  $Y_b$  represents a monovalent element or group selected from the class identified above in connection with  $Y$ ;  $b$  represents the number of  $Y$ 's and is equal to zero or a whole number corresponding to the valences on the nucleus  $T$  not satisfied with  $R^v$ ,  $(OM)$ , or  $(COOM')$ ; and  $n$  represents a whole number from one to four and indicates the total number of groups  $(T(OM)(COOM')Y_b)$  present in the molecule represented by the formula which

are attached to the aliphatic group or groups represented by  $R^v$  through the valences  $v$ .

In the foregoing general formula representation III it will be seen that the compounds represented thereby include those materials in which all of the aliphatic substituent is monovalent ( $v=1$  and  $n=1$ ) or in which all of the aliphatic substituent is polyvalent ( $v$  and  $n$  being equal to two, three, or four); or since  $R^v$  is defined as being at least one aliphatic radical or group and may therefore include several such groups, it will be seen that this general Formula III is inclusive of compounds having aliphatic groups or radicals of different valences (from one to four) in the same molecule. Also it will be observed that since  $n$  may be any whole number from one to four, the number of aromatic nuclei  $T$  in the molecule may likewise vary from one to four. It will be seen, therefore, that the relationship between  $n$  and  $v$  in Formula III, in its broadest aspect, is such that when  $n$  is equal to one,  $v$  is equal to one; and when  $n$  is greater than one, the valence  $v$  of at least one of the  $R^v$ 's is equal to  $n$  (in order to tie the several nuclei or  $T$ 's together), the valence of any remaining  $R^v$ 's being any whole number equal to or less than  $n$ .

As stated above and as will appear more fully later from the description of their synthesis, these materials represented by general Formula III may contain both monovalent and polyvalent aliphatic substituents. Both the polyvalent aliphatic substituent and the monovalent substituent, if both are present, may be introduced in the nucleus as part of an alkylation reaction, or all or part of the monovalent aliphatic substituent may be present in the nucleus of a hydroxy-aromatic starting material as low molecular weight aliphatic groups, such as methyl, ethyl, propyl groups, etc.

Compounds of the general type last described above, which include polyvalent substituted aliphatic substituents and may also include both the monovalent and the polyvalent substituents, are included under the subgeneric formula representation:

IV.  $R^v(T(OM)(COOM')Y_bR_c)_n$

in which  $T$ ,  $(OM)$ , and  $(COOM')$  have the same significance as indicated above;  $R^v$  represents at least one polyvalent aliphatic radical or group having a valence  $v$  of two, three, or four;  $Y_b$  indicates the same group of substituents as described above for  $Y$ ;  $R_c$  represents monovalent aliphatic radicals or groups;  $b$  represents the number of  $Y_b$ 's and is equal to zero or a whole number corresponding to the valences on the nucleus  $T$  not satisfied with  $R^v$ ,  $(OM)$ ,  $(COOM')$ , and  $R_c$ ;  $c$  indicates the number of  $R_c$ 's and is equal to zero or a whole number corresponding to the valences on the nucleus  $T$  not satisfied with  $R^v$ ,  $(OM)$ ,  $(COOM')$ , and  $Y_b$ ; and  $n$  represents a whole number from two to four and indicates the total number of the groups  $(T(OM)(COOM')Y_bR_c)$  present in the molecule represented by the formula which are attached to the aliphatic group or groups represented by  $R^v$  through the valences  $v$ .

In the above general Formulae III and IV it will be understood that since  $R^v$  and  $R^v'$  are aliphatic hydrocarbon radicals of the chain type and are each attached by one valence only to each corresponding aromatic nucleus, the valence  $v$  or  $v'$  of such radical or radicals is of necessity never greater than the number  $n$ , which indicates the number of aromatic nuclei in the molecule and in

Formula III is always equal to one when  $n$  equals one. Otherwise an  $R^v$  or an  $R^v'$  having a valence greater than the number ( $n$  or  $n'$ ) of aromatic nuclei would either have some of its valences unsatisfied or else would form a condensed ring or rings by attachment at two or more points to one and the same aromatic nucleus. Such latter compounds, as already indicated from the definition of  $R^v$  or  $R^v'$ , are not considered as characterizing the product of the present invention although probably formed in some instances in minor amounts as unobjectionable by-products by certain of the methods of preparation herein disclosed.

A simple type of compound coming under general Formula III in which  $v$  and  $n$  is each equal to one and in which there is only one oil-solubilizing aliphatic group  $R^v$  may be illustrated by the following formula showing  $T$  for purposes of illustration as a monocyclic nucleus:

A.



28

In the above formula the chain represents the oil-solubilizing alkyl substituent ( $R^v$ ), and  $Y_b$ ,  $(OM)$ , and  $(COOM')$ , have the same significance as has been heretofore given to these groups.

Since group  $R^v$  has been defined as "at least one", it will be apparent that there may be more than one heavy alkyl substituent attached to the nucleus  $T$ . Such a compound, where  $v$  and  $n$  are each one and in which there are two such monovalent  $R^v$  groups, may be represented by the following formula:

B.



45

in which the chains and the substituent characters have the same significance defined above.

Compounds of the type satisfying the general Formula III and the subgeneric Formula IV in which  $R^v$  (or  $R^v'$ ) is polyvalent and  $v$  (or  $v'$ ) and  $n$  (or  $n'$ ) are more than one and in which there is only one such polyvalent  $R^v$  group may be illustrated by the following formula, in which the aryl nucleus  $T$  is again indicated for illustration as being monocyclic:

C.



60

65

In the above formula C,  $R_c$  is a monovalent alkyl group as defined above under Formula IV and is the same as monovalent  $R^v$  in Formula III.

Under this same type of compound indicated by Formula C there may also be more than one polyvalent  $R^v$  group (represented by the chain) such a compound in which there are, for example, two polyvalent  $R^v$  groups being illustrated by the following formula, in which the

characterizing groups have the same significance described above under Formula C.



The possible molecular structure of compounds in which the aryl nucleus T is polycyclic will be obvious from the foregoing exemplary Formulae A to D, inclusive, and the possible molecular structure of compounds in which  $v$  and  $n$  are equal to two and four will be readily understood from the exemplary Formulae C and D.

15 Another possible molecular structure of compounds coming under general Formula III is a compound having more than one polyvalent  $R^v$ , at least two of which have different valences. Such a compound may be typified by the following formula in which the symbols have the same significance as in Formula C.



As to the possible number of  $R^v$  (and  $R_c$ ) groups going to make up a single molecule, this will vary with the extent to which it is desired to effect substitution of the nucleus with oil-solubilizing aliphatic groups for obtaining the desired properties in the product and is, of course, limited by the number of valences on the aromatic nucleus which are available for substitution. As will be apparent to those skilled in the art, the maximum possible number of  $R^v$  (and  $R_c$ ) groups which can be attached to a single aromatic nucleus will vary as the nucleus is mono or poly cyclic and also as the nucleus is otherwise substituted. It will also be apparent that available valences on the nuclei may all be attached to polyvalent aliphatic substituents.

It will be understood that the oil-improving agents contemplated by this invention may be pure compounds satisfying the general Formula III described above with any one of the various mono and poly cyclic aromatic nuclei as T and the various substituents  $R^v$  (or  $R^v$  and Y) described, the only requisites being that at least one nuclear hydrogen be substituted with a metal-oxy (OM) group, at least one nuclear hydrogen be substituted with a (COOM') group, and at least one nuclear hydrogen be substituted with an oil-solubilizing aliphatic radical or group. However, in manufacturing the preferred oil-improving product of the present invention by the preferred method of procedure, as will appear more fully later on, the final oil-improving product obtained is normally or usually a mixture of different compounds corresponding to different values of  $n$  and  $v$  and to different numbers of aliphatic groups  $R^v$ .

As has been emphasized hereinabove, it is important that the oil-improving agents as represented by general Formulae III and IV have

nuclear hydrogen in the aromatic nucleus T substituted with predominantly aliphatic material which comprises a sufficient proportion of the composition as a whole to render the same miscible with the mineral oil fraction in which the improving agent is used under normal conditions of handling and use. It appears from the results of our research that there is a critical range in the degree of alkylation of these improving agents below which the product or agent will not satisfy the requirements for oil-miscibility. Expressing this in another way, it appears that the hydroxyaromatic constituent of the alkylated hydroxyaromatic compound from which the alkylated metaloxyaromatic-metal carboxylate salt is derived should not exceed a certain percentage of such alkylated hydroxyaromatic composition as a whole. This critical range of alkylation may be roughly expressed as the ratio by weight of  $(T(OH))_n$  to  $R^v(T(OH))_n$ .

The degree of alkylation and the critical ranges within which operative and preferred compounds can be obtained may also be expressed as the number of carbon atoms contained in the aliphatic substituents for each aryl nucleus in a given molecule or molecular structure.

The critical range in the degree of alkylation of the aryl nucleus in the improving agents contemplated herein may vary with: (a) the mineral oil fraction in which the improving agent is to be used; (b) the aryl nucleus T (mono or poly cyclic); (c) the hydroxyl content of the aryl nucleus from which the final product is obtained (mono or polyhydric); (d) the character of aliphatic material comprising the substituent (straight or branched chain); (e) mono or poly substitution of the aryl nucleus; and (f) other substituents on the nucleus T, which may be of positive or negative or of neutral solubilizing activity.

In general it may be said that a polycyclic nucleus appears to require a higher degree of alkylation than a monocyclic nucleus; that a polyhydric nucleus requires a higher degree of alkylation than a monohydric nucleus; and that branched chain aliphatic substituents have a somewhat greater solubilizing action than straight chain solubilizing substituents.

In view of the foregoing variables it would be impracticable and probably misleading to attempt to give an expression and figure which would indicate accurately the proper ratio of hydroxyaromatic constituent to the alkylated hydroxyaromatic constituent which would express a degree of aliphatic substitution satisfying all cases taking these variables into account. As a guide for preparing these improving agents, however, our research indicates that for a product having poor depressing and V. I. improving properties in addition to other valuable properties the ratio, expressed as:

$$\text{VII. } \frac{(T(OH))_n}{R^v(T(OH))_n}$$

should not be greater than .17 when the weight of the hydroxyaromatic nucleus or component  $(T(OH))_n$  is expressed in terms of its chemically equivalent weight of phenol ( $C_6H_5OH$ ). However, for mere oil-solubility with inhibition of oxidation we have found that this ratio may be raised by poly-substituting the nucleus with branched chain aliphatic groups. In general it may be said that in the preferred improving agents contemplated herein the ratio by weight of the hydroxyaromatic component in the prod-

uct to the corresponding alkylated hydroxy-aromatic nucleus or component therein should not be greater than about seventeen parts by weight of the former to about 100 parts by weight of the latter, or about seventeen per cent, when the weight of the hydroxyaromatic nucleus or component is expressed in terms of its chemically equivalent weight of phenol. It will be observed that the ratio as represented by the 10 Formula VII does not take into account any other substituent in the nucleus than the aliphatic substituents and the hydroxyl group; but since the aliphatic substituent is primarily relied upon in the agents contemplated herein as 15 the solubilizing substituent, it is believed that the foregoing expression and limits will serve as a working guide for the preparation of oil-soluble materials and the preferred multifunctional materials.

20 As stated above, the degree of alkylation may also be expressed by the number of carbon atoms contained in the aliphatic substituent for a given hydroxyaromatic nucleus T. As a general guide here it may be said that the aliphatic substituents represented by R<sup>v</sup> in the above general Formula III should, for the preferred multifunctional materials contemplated herein, contain at least 25 thirty carbon atoms for each aromatic nucleus T.

The ratio of seventeen per cent, which we 30 may term the "phenolic ratio", represents what we consider a maximum figure for the preferred products contemplated herein, and in general it will be found that this figure will be lower, the actual ratio, of course, being dependent upon 35 the variable factors enumerated above. For example, as will later appear, an improving agent of the preferred type in which the aliphatic substituent is derived from petroleum wax (a predominantly straight chain aliphatic hydrocarbon 40 of at least twenty carbon atoms) and in which the aromatic nucleus was derived from phenol otherwise unsubstituted may have a phenolic ratio, as expressed above, not substantially greater than about thirteen per cent.

45 A further general guide for the synthesis of the preferred improving agents for viscous oils is to alkylate the aromatic nucleus so that it is polysubstituted with aliphatic hydrocarbon radicals or groups preferably of relatively high molecular weight.

50 As has been previously indicated, it is one of the primary objects of the invention to provide an oil-improving agent which will have multifunctional improving activity in a mineral oil. Our research indicates that compounds satisfying the requisites of general Formula III above 55 may be blended in minor proportions with mineral oil fractions, particularly of the viscous or lubricating oil type, to effect marked improvement in several important properties. The improvement effected may be varied somewhat with the aliphatic substituent, petroleum wax and aliphatic hydrocarbons of similar characteristics such as ester wax, for example, giving products 60 which effect a marked improvement in viscosity index and pour point in addition to other properties to be hereinafter pointed out. The effectiveness may also be varied with other substituents in the aryl nucleus—for example, alkoxy groups may contribute to solubility—and the 65 properties of the agents may also be varied with the character of the metal substituent in the carboxyl group. In general it appears that the oil-miscible salt of any metal satisfying the 70 requisites of Formula III above will act to inhibit

oxidation in mineral oils and reduce the formation of harmful oxidation products. Certain of the metals, such, for example, as lead and zinc, may serve to increase the load-carrying capacity of lubricating oils.

75 The procedure whereby the oil-improving agents contemplated by this invention can be prepared may be broadly described as follows:

First the hydroxyl hydrogen in an alkylated hydroxy-aromatic compound is substituted with an alkali or alkaline earth metal to form an alkylated aryl oxide of the corresponding alkali or alkaline earth metal which is then carboxylated to form the alkali or alkaline earth metal salt of the alkylated hydroxyaromatic carboxylic acid, the reactions being indicated by the following equation:



in which M<sup>a</sup> indicates an alkali or alkaline earth metal, and the remaining characters have the same significance described above in connection with general Formula III. If it is desired to obtain a metal oxyaromatic carboxylate salt in which the carboxyl hydrogen is replaced with alkali or alkaline earth metal the product of the above reactions may be used as an intermediate starting material for reaction (c) to be herein-after described.

When the desired product is one in which the carboxyl hydrogen is replaced with some metal other than an alkali or alkaline earth metal, the next step in the process involves substitution of the alkali or alkaline earth metal in the salt product of reaction (a) with the desired metal by a process of double decomposition, such reaction being indicated by the following equation:



in which M'X indicated an alcohol-soluble inorganic or fatty acid salt of the desired metal M'. In this double decomposition reaction, some of the metal may replace a nuclear hydrogen in the aromatic ring; but if such compounds form, they are in the minority and, in any event, are not considered harmful to the product.

To form the metal oxyaromatic-carboxylate salt from the hydroxyaromatic-metal carboxylate salt, the product from reaction (a) or (b) is reacted with an alcoholate or alkyl oxide of the desired metal, such reaction taking place according to the following equation:



in which "Alk(OM)" indicates the alcoholate of the metal M which may be the same as or different than the metal M'.

The metal substituents in the carboxyl group and the hydroxyl group of the improving agents described herein may be broadly classified as the metals belonging to the silver, copper, tin, aluminum, iron, alkali and alkaline earth analytical groups, which include: silver, mercury, lead, and thallium; bismuth, copper, and cadmium; arsenic, antimony, and tin; iron, cobalt, nickel, and manganese; barium, calcium, strontium, and magnesium; and sodium, potassium, and lithium, respectively. Other desirable metals include: titanium, cerium, thorium, vanadium, molybdenum, tungsten, uranium, and platinum.

The general reactions described and illustrated above, have shown an alkylated or an aliphatic-substituted hydroxyaromatic compound as the starting material. Compounds of this nature, which satisfy the requirements of high alkylation for the preferred improving agents discussed above, or mixtures of such compounds can be readily prepared by alkylating a mono or poly cyclic, mono or poly hydric, substituted or unsubstituted hydroxyaromatic compound with aliphatic compounds or predominantly aliphatic materials.

The starting material for the hydroxyaromatic constituent in the alkylation reaction to obtain an alkylated hydroxyaromatic product



in which  $Y_b$ , if present, is residual hydrogen, 20 may be a mono or poly cyclic hydroxyaromatic compound otherwise unsubstituted; or such compounds containing alkyl substituents; or in certain special cases (to be hereinafter described) the starting material may be an alkyl-aryl ether 25 or an aralkyl-aryl ether. For obtaining an alkylated hydroxyaromatic product containing a "Y" substituent, in addition to or in place of residual hydrogen, the starting material for the hydroxyaromatic constituent may be a mono or 30 poly cyclic hydroxyaromatic compound in which part of the nuclear hydrogen is substituted with a member or members of the group consisting of chlorine, hydroxy, alkoxy, aroxy, aryl, alkaryl, and aralkyl groups.

35 Examples of the hydroxyaromatic compounds which may be used as starting material for the alkylation reaction are: phenol, resorcinol, hydroquinone, catechol, cresol, xylanol, hydroxydiphenyl, benzylphenol, phenyl-ethyl-phenol, phenol resins, methyl-hydroxydiphenyl, guaiacol, alpha and beta naphthol, alpha and beta methyl naphthol, tolyl naphthol, xylol naphthol, benzyl naphthol, anthranol, phenyl methyl naphthol, phenanthrol, anisole, beta naphthyl methyl ether, chlorphenol, and the like. Preference in 45 general is to the monohydroxy phenols otherwise unsubstituted, particular preference being given to phenol and alpha and beta naphthol.

The alkylation of the hydroxyaromatic compound may be accomplished in various ways, such as by a Friedel-Crafts synthesis, using a halogenated aliphatic hydrocarbon, or by reaction with unsaturated high molecular weight aliphatic compounds or higher alcohols in the presence of 55  $H_2SO_4$  as a catalyst.

We have found the Friedel-Crafts type of alkylation reaction to be particularly adapted to the step of preparing the alkylated hydroxyaromatic compounds from which the improving agents described herein are synthesized because it affords a convenient means for controlling the degree of alkylation and obtaining the desired "phenolic ratio" for use in the preferred mineral oil compositions contemplated by this invention.

65 In this reaction an appropriate mono or poly chlorine-substituted aliphatic compound or material is reacted with the desired hydroxyaromatic compound in the presence of a catalytic amount of aluminum chloride. Pure or substantially pure mono or poly chlorine-substituted aliphatic compounds may be used. However, as will be readily understood by those skilled in the art, since it is usually very difficult to prepare or obtain high molecular weight aliphatic hydrocarbons in a pure or substantially pure state and

since it is equally difficult to prepare the chlorine (or other halogen) substitution products of such hydrocarbons in a pure or substantially pure state, we prefer to employ a mixture of such hydrocarbons, such as a suitable petroleum fraction, 5 as the starting material for our preferred improving agents, converting it into a mixture of different chlorine (or other halide) substitution products by any suitable method for use in the alkylation step. In general it may be said that the high molecular weight aliphatic hydrocarbons contemplated by this invention as preferred sources for the alkyl or aliphatic suhstituent  $R^v$  in Formula III above may be pure or mixed compounds typified by those which characterize the 15 heavier products of petroleum, such as heavy petroleum oils of the lubricant type, petrolatum, and crystalline petroleum wax or other compounds or materials which will result in relatively long chain aliphatic substituents. Special 20 preference is given to petroleum wax of melting point not substantially less than about 120° F. Such specially preferred aliphatic hydrocarbon materials commonly have molecular weights of about 250 and have at least twenty carbon atoms 25 in their molecules.

As stated above, the Friedel-Crafts synthesis affords a convenient means of controlling the "degree of alkylation" of the product. This is accomplished by controlling: (a) the chlorination 30 of the aliphatic hydrocarbon and (b) the reacting proportions of the chlorinated aliphatic hydrocarbon and the hydroxyaromatic compound used in the Friedel-Crafts reaction. As is well known to those skilled in the art, the replacement 35 of nuclear hydrogen in the hydroxyaromatic compound with an aliphatic group is, in the Friedel-Crafts synthesis, effected by reaction of such nuclear hydrogen with chlorine in the chlorinated aliphatic compound, the substitution 40 being effected with evolution of HCl. It will thus be seen that the number of chlorine substituents in a chlorinated aliphatic compound corresponds to the number of valences ( $v$  in general Formula III) which will be satisfied by or attached to 45 hydroxyaromatic nuclei in the product of the reaction. For example, in a reaction where a quantity of pure monochlor-aliphatic hydrocarbon containing say three atomic proportions of chlorine is reacted with one molecular proportion 50 of hydroxyaromatic compound, the resulting alkylated product,  $R^v(T(OH)Y_b)_n$ , is one in which  $v$  and  $n$  are equal to one and there are three aliphatic groups  $R^v$  attached to one nucleus T. On the other hand, assuming a reaction in which 55 a quantity of pure trichlor-aliphatic hydrocarbon containing three atomic proportions of chlorine is reacted with one molecular proportion of hydroxyaromatic compound, the product would be one in which  $v$  and  $n$  of general Formula III 60 are each equal to three, and the solubilizing action of a single aliphatic group would be distributed among three nuclear hydroxyaromatic groups. It is due to this latter condition that we consider it preferable that the number of valences " $v$ " 65 (in  $R^v$  of Formulae III, etc.) be maintained within the range of from one to four hereinabove specified. In other words, it appears that the required oil-solubilizing and oil-improving action of the aliphatic substituent  $R^v$ , particularly where 70 the aliphatic substituent is a wax derivative and the agent is to be used for multifunctional activity in viscous oils, is not obtained with materials predominantly comprised of a compound or compounds  $R^v(T(OM)(COOM')Y_b)_n$  (Formula III) 75

in which  $v$  and  $n$  are greater than four. Hence, for use in the Friedel-Crafts reaction the chlorinated high molecular weight aliphatic material should be a compound, or should be predominantly comprised of compounds in which the chlorine content is not greater than a tetrachlor compound.

As will be readily apparent to those skilled in the art, the chlorination of an aliphatic material such as a liquid petroleum fraction or a crystalline petroleum wax will normally or usually result in a mixture of mono- and poly-chlor-aliphatic hydrocarbon compounds. Consequently, the product of a Friedel-Crafts reaction between such chlorinated material and a hydroxyaromatic compound will be a mixture of different compounds corresponding to different values of  $v$  and  $n$  in the formula  $R^v(T(OH))_n$  and the final metal-oxyaromatic carboxylic acid salt derived therefrom according to the reaction of Equation c above will likewise be a mixture of compounds corresponding to different values of  $n$  and  $v$  in general Formula III. It will be understood, therefore, that the specific values for  $v$  and  $n$  in the above formula, as well as the formula itself, relate to the different specific compounds present in such a mixture which characterize it as a product of the present invention.

However, in the case of a pure compound corresponding to general Formula III or in mixtures thereof, we have, as previously stated, discovered that for a satisfactory product, the ratio by weight of hydroxyaromatic component  $(T(OH))_n$  to the corresponding alkylated hydroxyaromatic nucleus or component  $(R^v(T(OH))_n)$  should not be greater than a certain critical maximum ratio which varies with constituents, conditions of use, and properties desired, as discussed in detail hereinabove.

40 The above-mentioned ratio of hydroxyaromatic component to the corresponding alkylated hydroxyaromatic component

$$\left( \frac{(T(OH))_n}{R^v(T(OH))_n} \right)$$

45 in which the hydroxyaromatic component is calculated as phenol and which is therefore herein referred to as the phenol content or "phenolic ratio", is usually calculated from the weight of 50 the hydroxyaromatic compound used up in the alkylation reaction and from the total weight of alkylated compound resulting from such alkylation reaction, as will be readily understood by those skilled in the art.

55 For example, when the Friedel-Crafts synthesis is used for alkylation, the aliphatic hydrocarbon material is first chlorinated until the weight of chlorine absorbed indicates that the average composition of the chlorinated product corresponds roughly to say a dichlor-aliphatic hydrocarbon. Such a product will, of course, contain some mono- and tri-chlor compounds and probably some tetrachlor compounds. The reacting proportions (based on atomic proportions of chlorine to one mole of hydroxyaromatic compound) are then selected so that the theoretical product of the Friedel-Crafts reaction will give the approximate phenolic ratio desired. After the 60 Friedel-Crafts reaction and purification of the product the weight of aliphatic material in the chlorinated aliphatic starting material is subtracted from the weight of the alkylated or aliphatic-substituted product to obtain the weight 65 of hydroxyaromatic material  $((T(OH))_n)$  actu-

ally combined or used up in the alkylation synthesis. From this value and the weight of the alkylated product  $(R^v(T(OH))_n)$  the phenolic ratio or phenol content can be readily calculated. If there are other substituents ( $Y_b$ ) on the hydroxyaromatic nucleus in addition to the mono- or poly- valent aliphatic groups, a deduction should be made for them before calculating the phenolic ratio, an operation which will be apparent to those skilled in the art.

10 In the foregoing description of the Friedel-Crafts alkylation reaction we have referred to a hydroxyaromatic compound as a starting material. This same reaction may be used with an alkyl-aryl ether or an aralkyl-aryl ether which undergoes a substantial rearrangement during Friedel-Crafts alkylation to form an alkylated hydroxyaromatic compound in which the alkyl group of the ether replaces one of the nuclear 15 hydrogen atoms.

20 In the event it is desired to obtain a product  $R^v(T(OH))_n$  which contains an alkoxy group as the substituent  $Y_b$ , it is preferable that the alkylation be effected with a hydroxyaromatic compound containing such alkoxy or 25 aroxy group as a substituent and a high molecular weight unsaturated aliphatic hydrocarbon (such as polymerized isobutylene, dodecylene, tetradecene, octadecene, melene, etc.) or a higher alcohol (such as cetyl alcohol, myricyl 30 alcohol, ceryl alcohol, octadecyl alcohol, etc.) using  $H_2SO_4$  as a catalyst. By this procedure, the hydroxyaromatic ether can be alkylated without substantial rearrangement taking place. As an alternative procedure, polyhydric phenols 35 can be alkylated by reaction with alcohols or unsaturates or by Friedel-Crafts reaction follow by substitution of one hydroxy with a low molecular weight alkyl group. In carrying out this latter procedure, the alkylated polyhydric phenol is treated with an alkali alcoholate to introduce 40 alkali metal into the OH group followed by treating with the desired alkyl halide, whereby the substitution is effected.

45 When it is desired to obtain a nitro or amino group as the substituent "Y<sub>b</sub>" in general Formula III, the hydroxyaromatic compounds are alkylated when free of nitro or amino groups, and such alkylation is followed by nitration of the alkylated compound to introduce the nitro substituent. The amino group can be obtained by reduction of the nitro group.

#### PREPARATION OF METALOXYAROMATIC-METAL CARBOXYLATE SALTS FROM WAX-SUBSTITUTED PHENOL

55

##### (1) Alkylation of phenol

A paraffin wax melting at approximately 120° F. and predominantly comprised of compounds having at least twenty carbon atoms in their molecules is melted and heated to about 200° F., after which chlorine is bubbled therethrough until the wax has absorbed from sixteen per cent to twenty per cent of chlorine, such product having an average composition between a monochlor wax and a dichlor wax or corresponding roughly to a dichlor wax. Preferably the chlorination is continued until about one-sixth the weight of the "chlorwax" formed is chlorine. A quantity of 60 chlorwax thus obtained, containing three (or four, with twenty per cent chlorine in the chlorwax) atomic proportions of chlorine, is heated to a temperature varying from just above its melting point to not over 150° F., and one mole 65 of hydroxyaromatic material  $((T(OH))_n)$  actu-

75

of phenol ( $C_6H_5OH$ ) is admixed therewith. The mixture is heated to about 150° F., and a quantity of anhydrous aluminum chloride corresponding to about three per cent of the weight of chlorwax in the mixture is slowly added to the mixture with active stirring. The rate of addition of the aluminum chloride should be sufficiently slow to avoid violent foaming, and during such addition the temperature should be held at about 150° F. 5

10 After the aluminum chloride has been added, the temperature of the mixture may be increased slowly over a period of from fifteen to twenty-five minutes to a temperature of about 250° F. and then should be more slowly increased to about 15 350° F. To control the evolution of HCl gas the temperature of the mixture is preferably raised from 250° F. to 350° F. at a rate of approximately one degree per minute, the whole heating operation occupying approximately two hours from the 20 time of adding the aluminum chloride. If the emission of HCl gas has not ceased when the final temperature is reached, the mixture may be held at 350° F. for a short time to allow completion of the reaction. But, to avoid possible 25 cracking of the wax, the mixture should not be heated appreciably above 350° F., nor should it be held at that temperature for any extended length of time.

It is important that all unreacted or non- 30 alkylated hydroxyaromatic material (phenol) remaining after the alkylation reaction be removed. Such removal can be effected generally by water-washing, but it is preferable to treat the water-washed product with super-heated steam, thereby 35 insuring complete removal of the unreacted material and accomplishing the drying of the product in the same operation.

The wax-substituted phenol thus obtained may be characterized by the general formula 40  $R^v(T(OH)Y_b)_n$ , in which  $R^v$  represents at least one aliphatic group or radical characteristic of paraffin wax having a valence  $v$  of from one to four;  $T$  represents a monocyclic aromatic nucleus;  $Y_b$  represents residual hydrogen,  $b$  being a number corresponding to the number of 45 valences on the nucleus  $T$  not satisfied by  $R^v$  and  $(OH)$ ; and  $n$  as a number from one to four corresponding to the valences  $v$  on the aliphatic group or groups  $R^v$  which are satisfied by the 50 nuclear group or groups  $T(OH)Y_b$ . At this step of the process,  $b$  in the above general formula should always be at least one, since residual hydrogen in the nucleus is important to the carboxylation step to be hereinafter described.

55 A wax-substituted phenol prepared according to the above procedure, in which a quantity of chlorwax containing three atomic proportions of chlorine (sixteen per cent chlorine in the chlorwax) is reacted with one mole of phenol, may, for brevity herein, be designated as "wax-phenol 60 (3-16)." Parenthetical expressions of this type (A-B) will be used hereinafter in connection with the alkylated hydroxyaromatic compounds to designate (A) the number of atomic proportions of chlorine in chlor-aliphatic material reacted with one mole of hydroxyaromatic compound in the Friedel-Crafts reaction, and (B) the chlorine content of the chlor-aliphatic material. In the above example A=3 and B=16. This 65 same designation will also apply to the metal-hydroxyaromatic-metal carboxylate derivatives.

70 Wax-phenol (3-16) as obtained by the above procedure had a phenol content or a "phenolic ratio" of about thirteen per cent and wax phenol (4-20) had a "phenolic ratio" of about 12.5 per

cent. Our research indicates that this phenolic ratio in the neighborhood of thirteen per cent may be considered as representing about the maximum for satisfactory miscibility and multifunctional activity in viscous oils of the metal-hydroxyaromatic-metal carboxylate derivatives of alkylated hydroxyaromatic compounds in which the alkyl substituent is derived from wax and the hydroxyaromatic constituent is derived from phenol ( $C_6H_5OH$ ).

(2) *Formation of wax-substituted alkali or alkaline earth metal phenate*

As an example of this step in the preparation of our oil-improving agents, wax-substituted sodium phenate can be prepared by the reaction of wax-phenol with metallic sodium in the presence of a non-oxidizing gas. The reaction mixture is heated at 500° F. during a two-hour period with rapid stirring to produce finely divided sodium and thereby accelerate the reaction. The proportions of reactants which were used in preparing a wax-substituted alkali metal phenate according to the above procedure were:

|                                                    | Grams |
|----------------------------------------------------|-------|
| Wax-phenol (13.2 per cent combined phenol content) | 500   |
| Sodium or equivalent amount of potassium           | 16    |

Wax-substituted phenates of the alkali and alkaline earth metals may also be prepared by reacting a wax-phenol with the desired alcoholate or alkyl metal oxide of an alkali or alkaline earth metal. For this purpose anhydrous methyl and ethyl alcohols are usually most suitable for use in preparing the alkyl metal oxides. As an example, 500 grams of wax-phenol (3-16) of 13.2 per cent combined phenol content was reacted with sixteen grams of sodium in the form of the ethyl sodium oxide by heating the mixture to about 300° F. during a one-hour period and allowing the alcohol released in the reaction to distill off, thereby obtaining the wax-substituted sodium phenate as the final product.

(3) *Carboxylation to form alkali or alkaline earth metal salt of wax-phenol carboxylic acid*

A product of the foregoing step, such as the wax-substituted sodium phenate, is heated to a temperature of about 350° F., and  $CO_2$  is introduced at a rate sufficient to maintain this temperature. The pressure is gradually raised to about 500 pounds per square inch to complete the reaction at this temperature during a one-hour period. The reaction may be illustrated with unsubstituted sodium phenate by the following equations:



By rearrangement the carboxy group is transferred to the ring, giving the sodium salt of the phenol carboxylic acid:



Other carboxylating reactions may be used in this step of the process, such as the reaction of

the alkali metal wax-phenate with carbonyl chloride or carbon tetrachloride; but since the acid salt formed in the presence of  $\text{CO}_2$  is obtained in high yield and in a pure state, this is the preferred carboxylation procedure.

Because of the high viscosity of the mixture it is advantageous to dilute the wax-substituted phenol initially with one or two parts of mineral oil. When a diluent has been used, carbon dioxide can be introduced at room temperature; and the temperature of the reaction in this case may be regulated by the amount of external heating.

The product of this step, where the starting material was wax-substituted sodium phenate, is the sodium salt of wax-substituted phenol carboxylic acid.

(4) *Formation of the salts of other metals*

With an alkali or alkaline earth metal salt, such as the sodium salt of the foregoing step, as the starting material, the corresponding salts of the other metals can be prepared by double decomposition of the first-mentioned salt with an alcohol-soluble inorganic or fatty acid salt of the desired metal. The use of alcohol as a solvent for the salt is desirable to insure proper solution and reaction, the reaction being conveniently carried out by heating the mixture at 175° F. during a two-hour period.

The reaction product of this double decomposition or the alkali or alkaline earth metal salt obtained in the previous step is used as an intermediary for obtaining the final metaloxyaromatic-metal carboxylate salt contemplated by this invention.

The reaction mixture employed in this double decomposition reaction may, for example, consist of one mole of the sodium salt of wax-substituted phenol carboxylic acid and one mole equivalent of the inorganic or fatty acid salt of the desired metal in alcohol solution. One part by volume of Stoddard solvent may be employed as a diluent for the mixture.

(5) *Formation of the metaloxyaromatic-metal carboxylate type of salt*

As illustrated by equation (c) above the salts of Formula III are obtained by replacing the hydroxyl hydrogen with the desired metal which may be the same as or different from the metal on the carboxyl group.

The substitution of the hydroxyl hydrogen in the salt of the hydroxyaromatic (phenol carboxylic) acid obtained in steps (3) or (4) described above is obtained by reacting such salt with an alcoholate or alkyl oxide of the desired metal. The alkyl oxides may be conveniently formed by double decomposition of alkyl sodium oxide with an alcohol-soluble salt (such as a chloride) of the desired metal to form the metal alcoholate and the inorganic sodium salt.

The alkyl-substituted hydroxyaromatic acid salt may be added to the alkyl metal oxide mixture without separating the sodium salt (chloride) from the pure alkyl metal oxide. The mixture is heated during a one-hour period at 300° F., allowing the alcohol to distill to complete the formation of the metaloxyaromatic-metal carboxylate salt (Formula III). The product thus obtained is separated from the inorganic reaction salts, which are insoluble, by settling, filtering, or centrifuging, without resorting to water-washing. If desired, the reaction mixture prior to separation, may be diluted with a suitable solvent such as a light mineral oil to

aid the separation of the salt, such separation being followed by distillation of the diluent to obtain the finished material.

It is to be understood that the foregoing procedure is merely illustrative of the methods which may be employed in synthesizing the various metaloxyaromatic-metal carboxylate salts of alkylated hydroxyaromatic acids contemplated by this invention; that polycyclic hydroxyaromatic compounds may be used instead of phenol and that other aliphatic compounds or predominantly aliphatic materials may be used as the source of the solubilizing alkyl or aliphatic substituent ( $\text{R}'$ ) in general Formula III.

As will appear from the foregoing description, the oil-improving agents contemplated by this invention are characterized by the general Formula III ( $\text{R}'(\text{T}(\text{OM})(\text{COOM}')\text{Y}_b)_n$ ) described hereinabove, such compounds or products may also be characterized as oil-miscible alkylated or alkyl-substituted hydroxyaromatic carboxylic acids in which the hydroxyl and carboxyl hydrogens have been substituted with their equivalent weight of metal; also as the metal salts of alkylated metaloxyaromatic carboxylic acids, it being understood that the terms "alkyl" and "alkylated" are used herein in a broad sense to include polyatomic or polyvalent, as well as monovalent aliphatic radicals or groups.

To demonstrate the effectiveness of compounds or products of the type described above in the mineral oil compositions contemplated by this invention, we have conducted several comparative tests, the results of which are listed below, with representative mineral oils alone and with the same oils blended with the improving agents contemplated by this invention.

The improving agents used in these tests included salts of the type above described in which both the carboxyl and hydroxyl hydrogens were substituted with the same metal and salts in which the carboxyl and hydroxyl hydrogens were substituted with different metals. Salts of the former type are designated as "di" salts, for example dicobaltous salt of wax phenolic acid or di-cobaltous (phenate-carboxy) salts of wax phenolic acid. In referring to salts of the latter type the hydroxyl metal substituent is indicated with the suffix (OM) and the carboxyl metal substituent is indicated with the suffix (COOM'). Thus, for example, a salt of wax-substituted phenol carboxylic acid in which the hydroxyl hydrogen is substituted with copper and the carboxyl hydrogen is substituted with sodium will be referred to and indicated in the tables as the cupric (OM)-sodium (COOM') salt of wax phenol carboxylic acid.

SLUDGE INHIBITION

This series of tests was conducted with mineral lubricating oil having a Saybolt viscosity of 244 seconds at 130° F. The test involved subjecting the oil and various oil blends to accelerated oxidizing conditions in the presence of metal at a temperature of 350° F. over an extended period of time, the amount of sludge formed during such test being expressed as the tar number. The improving agents used were prepared according to the procedure outlined hereinabove. The comparative results obtained are indicated in the table below, in which it will be observed that the metaloxyaromatic-metal carboxylate salts are effective to substantially stabilize the oil against the formation of sludge under these highly accelerated oxidizing conditions.

Table I

| 5  | Inhibitor blended with motor oil of Saybolt viscosity of 244 sec. @ 130° F. | Concen. by weight | Tar numbers on oil blends evaluated at 350° F. |        |         |         |         |
|----|-----------------------------------------------------------------------------|-------------------|------------------------------------------------|--------|---------|---------|---------|
|    |                                                                             |                   | Start                                          | 7 days | 10 days | 11 days | 14 days |
| 10 | None                                                                        | Percent           | 0                                              | 18     |         |         |         |
|    | Cuprite(OM)-sodium (COOM') salt of wax phenol carboxylic acid               | 1/4               | 0                                              | 0      | 0       | 0.2     |         |
|    | Disodium salt of wax phenol carboxylic acid                                 | 1/4               | 0                                              | 0      | 0       | Viscous |         |
| 15 | Cobaltous (OM)-manganese (COOM') salt of wax phenol carboxylic acid         | 1/4               | 0                                              | Trace  |         |         |         |
|    | Distannous salt of wax phenol carboxylic acid                               | 1/4               | 0                                              | Trace  |         |         |         |
| 20 | Dicobaltous salt of wax phenol carboxylic acid                              | 1/4               | 0                                              | Trace  |         |         |         |
|    | Diferrie salt of wax phenol carboxylic acid                                 | 1/4               | 0                                              | Trace  |         |         |         |
|    |                                                                             | 1/4               | 0                                              | 0      | 0       | Viscous |         |

## 25 POUR POINT DEPRESSION

In addition to the property of inhibiting sludge formation the metal oxyaromatic-metal carboxylate salts of wax-substituted hydroxyaromatic acids are effective pour point depressants, as indicated by the results tabulated below. These results were obtained from blends of mineral lubricating oil having a Saybolt Universal viscosity of 244 seconds at 130° F. and containing metal salts of the metaloxy-metal carboxylate type derived from wax-substituted phenol and prepared according to the procedure outlined above. The pour point of the oil alone was 20° F., and as is clearly indicated by Table II below, the salts contemplated by this invention are effective in very small amounts to reduce the pour point as much as 40° F.

Table II

| 45 | Depressant blended with motor oil of Saybolt viscosity of 244 sec. @ 130° F. | A. S. T. M. pour tests on oil blends |      |      |
|----|------------------------------------------------------------------------------|--------------------------------------|------|------|
|    |                                                                              | 0%                                   | 1/2% | 1/8% |
| 50 | None                                                                         | °F.                                  |      |      |
|    | Cuprite(OM)-sodium (COOM') salt of wax phenol carboxylic acid                | +20                                  |      |      |
|    | Disodium salt of wax phenol carboxylic acid                                  |                                      | -10  | -20  |
|    | Cobaltous (OM)-manganese (COOM') salt of wax phenol carboxylic acid          |                                      | -10  | -20  |
|    | Distannous salt of phenol carboxylic acid                                    |                                      | -5   | -15  |
| 55 | Dicobaltous salt of phenol carboxylic acid                                   |                                      | -10  | -25  |
|    | Diferrie salt of phenol carboxylic acid                                      |                                      | -10  | -20  |
|    |                                                                              |                                      | -10  | -20  |

## OPERATION TEST

In addition to the foregoing tests we have also made tests of an oil and an oil blend containing a representative improving agent of the type contemplated by this invention to determine the comparative behavior of the unblended oil and the improved oil under actual operating conditions. The test was carried out in a single cylinder C. F. R. engine. The engine was operated continuously over a time interval of twenty-eight hours, with the cooling medium held at a temperature of about 390° F., at a speed of 1200 R. P. M., which is equivalent to a road speed of about twenty-five miles per hour. The oil temperature was held at about 150° F., during the test.

The oil used in this test was a lubricating oil stock of 120 seconds Saybolt Universal viscosity

at 210° F., and the conditions observed at the end of the test were (a) the extent to which the piston rings were stuck, (b) the extent to which the slots in the oil rings were filled with deposit, (c) the amount of carbonaceous deposits in the oil, and (d) the acidity or neutralization number (N. N.) of the oil at the end of the test. The "oil" indicated as "A" in Table III below is the unblended oil and oil "B" is the same oil containing 1/4% of dicobaltous (phenate-carboxy) salt of wax phenolic acid.

Table III

| Oil | Ring condition |     |     |     |     | Carbon deposit | N.N. |  |  |
|-----|----------------|-----|-----|-----|-----|----------------|------|--|--|
|     | Degrees stuck  |     |     |     |     |                |      |  |  |
|     | 1              | 2   | 3   | 4   | 5   |                |      |  |  |
| A   | 90             | 360 | 360 | 360 | 360 | 20             | 80   |  |  |
| B   | 60             | 0   | 45  | 0   | 0   | 0              | 5    |  |  |

From the foregoing results it will be apparent that metal oxyaromatic-metal carboxylate salts of the type contemplated by this invention are effective oil-improving agents and are characterized by the fact that they have, through the presence of the metal substituents, multi-functional activity. Although we do not wish to be bound in any regard by any theory as to the function which the metal substituents have, it is believed that such substituents act by promoting the preferential oxidation of the alkylated hydroxyaromatic acid molecule, thereby taking up active oxygen and acting as a direct antioxidant; also by acting as a peptizing agent on any sludge that is formed in the oxidation of the oil; and in the event an alkali or alkaline earth metal is present as one or all of the metal substituents the salts act by neutralizing strong acids in the oil, particularly sulfur acids, such as may be formed by oxidation. The improved properties obtained and the degree of improvement in a particular property may be varied with the metal substituents, the aryl constituents, and the degree of alkylation of the aryl nucleus.

As to the degree of alkylation, it is important that the aryl nucleus be sufficiently alkylated to provide a final product which is "soluble" or "miscible" in the particular mineral oil fraction with which it is to be blended, that is, one which will remain uniformly dispersed in the oil in sufficient amount to effect the desired improvement, under normal conditions of storage and use.

The amount of improving agent used may be varied, depending upon the mineral oil or the mineral oil fraction with which it is blended and the properties desired in the final oil composition. The metal oxyaromatic-metal carboxylate salts of the type described herein may be used in amounts ranging from one-sixteenth per cent to ten per cent, and, in general, compositions of the desired improved properties may be obtained with these improving agents in amounts of from one-sixteenth per cent to two per cent.

It is to be understood that while we have described certain preferred procedures which may be followed in the preparation of the metal oxyaromatic-metal carboxylate salts of alkylated hydroxyaromatic acids used as improving agents in the mineral oil compositions contemplated by this invention and have referred to various representative constituents in these improving agents,

such procedures and examples have been used for illustrative purposes only. The invention, therefore, is not to be considered as limited by the specific examples given but includes within its scope such changes and modifications as fairly come within the spirit of the appended claims.

We claim:

1. An improved mineral oil composition comprising a mineral oil having admixed therewith a minor proportion of an oil-miscible metaloxy-aromatic-metal carboxylate salt in which part of the hydrogen of the aromatic nucleus has been replaced with a mineral oil solubilizing substituent.
2. An improved mineral oil composition comprising a mineral oil having admixed therewith a minor proportion of an oil-miscible metaloxy-aromatic-metal carboxylate salt in which part of the hydrogen of the aromatic nucleus has been substituted with predominantly aliphatic organic material, said last-mentioned substituent comprising a sufficient proportion of the substituted metaloxyaromatic-metal carboxylate salt to render such salt miscible with said oil under normal conditions of handling and use.
3. An improved mineral oil composition comprising a mineral oil having admixed therewith in minor proportion: an oil-miscible wax-substituted metaloxyaromatic compound having at least one hydrogen atom on the aryl nucleus substituted with a carboxyl group in which the carboxyl hydrogen is replaced with its equivalent weight of metal.
4. An improved mineral oil composition comprising a mineral oil having admixed therewith a minor proportion of an oil miscible metal salt of an alkyl-substituted hydroxyaromatic carboxylic acid in which both the hydroxyl hydrogen and the carboxyl hydrogen are substituted with metal.
5. An improved mineral oil composition comprising a mineral oil having admixed therewith a minor proportion of an oil-miscible metal salt of an alkyl-substituted hydroxyaromatic carboxylic acid in which both the hydroxy hydrogen and the carboxyl hydrogen are substituted with the same metal.
6. An improved mineral oil composition comprising a mineral oil having admixed therewith a minor proportion of an oil-miscible metal salt of an alkyl-substituted hydroxyaromatic carboxylic acid in which the hydroxyl hydrogen and the carboxyl hydrogen are substituted with different metals.
7. An improved mineral oil composition comprising a mineral oil having admixed therewith a minor proportion of an oil-miscible metal salt of an alkyl-substituted hydroxyaromatic carboxylic acid in which both the hydroxyl hydrogen and the carboxyl hydrogen are substituted with metal and in which the alkyl substituent comprises a high molecular weight hydrocarbon derivative.
8. An improved mineral oil composition comprising a mineral oil having admixed therewith a minor proportion of an oil-miscible metal salt of an alkyl-substituted hydroxyaromatic carboxylic acid in which both the hydroxyl hydrogen and the carboxyl hydrogen are substituted with metal and in which the alkyl substituent is derived from an aliphatic hydrocarbon having at least twenty carbon atoms.
9. An improved mineral oil composition comprising a mineral oil having admixed therewith a minor proportion of an oil-miscible metal salt of an alkyl-substituted hydroxyaromatic car-

boxylic acid in which both the hydroxyl hydrogen and the carboxyl hydrogen are substituted with metal and in which the alkyl substituent is derived from petroleum wax.

10. An improved mineral oil composition comprising a mineral oil having admixed therewith a minor proportion of an oil-miscible metal salt of an alkyl-substituted hydroxyaromatic carboxylic acid in which both the hydroxyl hydrogen and the carboxyl hydrogen are substituted with metal, the alkyl substituent in said salt being a high molecular weight aliphatic hydrocarbon derivative and the aryl nucleus being poly-substituted with said aliphatic derivative.

11. An improved mineral oil composition comprising a mineral oil having admixed therewith a minor proportion of an oil-miscible metal salt of an alkyl-substituted hydroxyaromatic carboxylic acid in which both the hydroxyl hydrogen and the carboxyl hydrogen are substituted with metal, the alkyl substituent in said salt being derived from an aliphatic hydrocarbon having at least twenty carbon atoms and the aryl nucleus thereof being poly-substituted with said aliphatic derivative.

12. An improved mineral oil composition comprising a mineral oil having admixed therewith a minor proportion of an oil-miscible metal salt of an alkyl-substituted hydroxyaromatic carboxylic acid in which both the hydroxyl hydrogen and carboxyl hydrogen are substituted with metal, the alkyl substituent in said salt being a derivative of petroleum wax and the aryl nucleus thereof being poly-substituted with said wax derivative.

13. An improved mineral oil composition comprising a mineral oil having admixed therewith a minor proportion of an oil-miscible metal salt of an alkyl-substituted phenol-carboxylic acid in which both the hydroxyl hydrogen and the carboxyl hydrogen are replaced with metal.

14. An improved mineral oil composition comprising a mineral oil having admixed therewith a minor proportion of an oil-miscible metal salt of an alkyl-substituted phenol-carboxylic acid in which both the hydroxyl hydrogen and the carboxyl hydrogen are replaced with metal, the alkyl substituent in said salt being a high molecular weight aliphatic hydrocarbon derivative.

15. An improved mineral oil composition comprising a mineral oil having admixed therewith a minor proportion of an oil-miscible metal salt of an alkyl-substituted phenol-carboxylic acid in which both the hydroxyl hydrogen and the carboxyl hydrogen are replaced with metal, the alkyl substituent in said salt being a high molecular weight aliphatic hydrocarbon derivative and the aryl nucleus thereof being poly-substituted with said aliphatic derivative.

16. An improved mineral oil composition comprising a mineral oil having admixed therewith a minor proportion of an oil-miscible metal salt of an alkyl-substituted phenol-carboxylic acid in which both the hydroxyl hydrogen and the carboxyl hydrogen are replaced with metal, the alkyl substituent in said salt being a derivative of petroleum wax.

17. An improved mineral oil composition comprising a mineral oil having admixed therewith a minor proportion of an oil-miscible metal salt of an alkyl-substituted phenol-carboxylic acid in which both the hydroxyl hydrogen and the carboxyl hydrogen are replaced with metal, the alkyl substituent in said salt being a derivative of

5

10

15

20

25

30

35

40

45

50

55

60

65

70

75

petroleum wax and the aryl nucleus thereof being poly-substituted with said wax derivative.

18. An improved mineral oil composition comprising a mineral oil having admixed therewith a minor proportion of a metal salt of a carboxylated-alkylated phenol in which the hydroxyl hydrogen and the carboxyl hydrogen are substituted with metal, the alkyl substituent being derived from petroleum wax and the proportion 5 by weight of phenol in the parent alkylated-phenol constituent being in the neighborhood of thirteen per cent.

19. An improved mineral oil composition comprising a mineral oil having admixed therewith a minor proportion of a metal salt of a carboxylated-alkylated hydroxyaromatic compound in which the hydroxyl hydrogen and the carboxyl hydrogen are substituted with metal, the alkyl substituent thereof being a derivative of petroleum wax and the proportion by weight of the hydroxyaromatic constituent in the parent alkylated - hydroxyaromatic constituent being chemically equivalent to not more than about seventeen per cent phenol.

20. An improved mineral oil composition comprising a mineral oil having admixed therewith a minor proportion of an oil-soluble metal salt of an alkyl-substituted hydroxyaromatic carboxylic acid in which the hydroxyl hydrogen and the carboxyl hydrogen are substituted with metal, said metal substituents being selected from metals of the silver, copper, tin, aluminum, iron, alkaline earth and alkali analytical groups.

21. An improved mineral oil composition comprising a mineral oil having admixed therewith a minor proportion of a product of the type obtained by: chlorinating petroleum wax until about one-sixth of the reaction product is chlorine; reacting the chlorinated wax with a hydroxyaromatic compound in the proportion of one mol of the latter to an amount of the chlorinated wax containing about three atomic proportions of chlorine to form a wax-substituted hydroxyaromatic compound; substituting the hydroxyl hydrogen thereof with metal to form a wax-substituted aryl metal oxide of said metal; carboxylating said metal oxide to form a metal salt of a wax-substituted hydroxyaromatic carboxylic acid; and substituting the hydroxyl hydrogen of said salt with a metal.

22. An improved mineral oil composition comprising a viscous mineral oil fraction having admixed therewith a minor proportion, from about one-sixteenth to about ten per cent of an oil-miscible alkyl - substituted metaloxyaromatic metal carboxylate salt.

23. An improved mineral oil composition comprising a viscous mineral oil fraction having admixed therewith a minor proportion, from about one-sixteenth to about ten per cent of an oil-miscible alkyl - substituted metaloxyaromatic metal carboxylate salt in which the alkyl substituent is derived from an aliphatic hydrocarbon having at least twenty carbon atoms.

24. An improved mineral oil composition comprising a viscous mineral oil fraction having admixed therewith a minor proportion, from about one-sixteenth to about ten per cent of an oil-miscible alkyl - substituted metaloxyaromatic metal carboxylate salt in which the alkyl substituent is derived from petroleum wax.

25. A composition of matter comprising a mineral oil fraction and in admixture therewith a minor proportion of an oil miscible metalorganic compound having the general formula:

$R^v(T(OM)(COOM')Y_b)_n$

in which: T represents an aromatic nucleus; (OM) represents at least one hydroxyl group in which the hydroxyl hydrogen is replaced with its equivalent weight of a metal M, said group being attached to the nucleus T; (COOM') is attached to the nucleus T and represents at least one carboxyl group the hydrogen of which is replaced by its equivalent weight of a metal M'; R<sup>v</sup> represents at least one aliphatic group having a valence V of one to four, and is attached by one valence only to at least one nucleus T; Y represents a monovalent radical selected from the group consisting of residual hydrogen, and chlorine, alkoxy, 15 aroxy, aralkyl, alkaryl, aryl, nitro and amino radicals; b represents the number of Y's and is equal to zero or a whole number corresponding to the valences on the nucleus T not satisfied by R<sup>v</sup>, (OM), or (COOM'); and n is a whole number from one to four; the substituent R<sup>v</sup> comprising a sufficient proportion of the metalorganic compound to render same miscible with said oil under normal conditions of handling and use.

26. A composition of matter comprising a mineral oil fraction and in admixture therewith a minor proportion of an oil-miscible metalorganic compound having the general formula

$R^v(T(OM)(COOM')Y_b)_n$

in which: T represents an aromatic nucleus; (OM) represents at least one hydroxyl group in which the hydroxyl hydrogen is replaced by its equivalent weight of a metal M, said group being attached to the nucleus T; (COOM') is attached to the nucleus T and represents at least one carboxyl group the hydrogen of which is replaced by its equivalent weight of a metal M'; R<sup>v</sup> represents at least one aliphatic group having a valence v, of one to four, and attached by one valence only to at least one nucleus T; Y represents a monovalent radical selected from the group consisting of residual hydrogen, and chlorine, alkoxy, aroxy, aralkyl, alkaryl, aryl, nitro, and amino radicals; b represents the number of Y's and is equal to zero or a whole number corresponding to the valences on the nucleus T not satisfied by R<sup>v</sup>, (OM) or (COOM') and n is a whole number from one to four; the total number of carbon atoms in all of the aliphatic groups taken together in said metalorganic compound being not less than about 50 thirty for each nucleus T.

27. A composition of matter comprising a mineral oil fraction and in admixture therewith a minor proportion of an oil-miscible metalorganic compound having the general formula:

$R^v(T(OM)(COOM')Y_b)_n$

in which: T represents an aromatic nucleus; (OM) represents at least one hydroxyl group in which the hydroxyl hydrogen is replaced with its equivalent weight of metal M, said group being attached to the nucleus T; (COOM') is attached to the nucleus T and represents at least one carboxyl group the hydrogen of which is replaced by its equivalent weight of a metal M'; R<sup>v</sup> represents at least one aliphatic group having a valence v, of one to four, and attached by one valence only to at least one nucleus T; Y represents a monovalent radical selected from the group consisting of residual hydrogen, and chlorine, alkoxy, aroxy, aralkyl, alkaryl, aryl, nitro, and amino radicals; b represents the number of Y's and is equal to zero or a whole number corresponding to the valences on the nucleus T not satisfied by R<sup>v</sup>, (OM) or (COOM'); and n is a whole number 75

from one to four; the equivalent ratio of  $T(OH)$  to  $R'(T(OH))_n$  in said metalorganic compound being not greater than the chemical equivalent of twenty per cent phenol.

5 28. A composition of matter comprising a mineral oil fraction and in admixture therewith a minor proportion of an oil-miscible metalorganic compound having the general formula:



10 in which: T represents an aromatic nucleus; (OM) represents at least one hydroxyl group in which the hydroxyl hydrogen is replaced with its equivalent weight of metal M, said group being attached to the nucleus T; (COOM') is attached to the nucleus T and represents at least one carboxyl group the hydrogen of which is replaced by its equivalent weight of metal M'; R'' represents at least one polyvalent aliphatic hydro-

carbon group of at least twenty carbon atoms having a valence  $v'$  of from two to four;  $Y_b$  represents a monovalent radical selected from the group consisting of residual hydrogen, chlorine, alkoxy, aroxy, aralkyl, aryl, nitro, and amino radicals;  $b'$  represents the number of  $Y_b$ 's and is equal to zero or a whole number corresponding to the valences on the nucleus T not satisfied by  $R''$ , (OM), (COOM') and  $R_c$ ;  $R_c$  represents monovalent aliphatic radicals;  $c$  10 represents the number of  $R_c$ 's and is equal to zero or a whole number corresponding to the valences on the nucleus T not satisfied by  $R''$ , (OM), (COOM') and  $Y_b$ ; and  $n$  is a whole number from two to four. 15

ORLAND M. REIFF.  
JOHN J. GIAMMARIA.  
HORACE E. REDMAN.